



US010213837B2

(12) **United States Patent**  
**Kondoh**

(10) **Patent No.:** **US 10,213,837 B2**  
(45) **Date of Patent:** **Feb. 26, 2019**

(54) **TITANIUM POWDER CONTAINING SOLID-SOLUTED NITROGEN, TITANIUM MATERIAL, AND METHOD FOR PRODUCING TITANIUM POWDER CONTAINING SOLID-SOLUTED NITROGEN**

(71) Applicants: **HI-LEX CORPORATION**, Hyogo (JP); **Katsuyoshi Kondoh**, Osaka (JP)

(72) Inventor: **Katsuyoshi Kondoh**, Osaka (JP)

(73) Assignees: **HI-LEX CORPORATION**, Hyogo (JP); **KATSUYOSHI KONDOH**, Osaka (JP)

(\*) Notice: Subject to any disclaimer, the term of this patent is extended or adjusted under 35 U.S.C. 154(b) by 163 days.

(21) Appl. No.: **15/113,637**

(22) PCT Filed: **Dec. 26, 2014**

(86) PCT No.: **PCT/JP2014/084530**

§ 371 (c)(1),

(2) Date: **Jul. 22, 2016**

(87) PCT Pub. No.: **WO2015/111361**

PCT Pub. Date: **Jul. 30, 2015**

(65) **Prior Publication Data**

US 2017/0008087 A1 Jan. 12, 2017

(30) **Foreign Application Priority Data**

Jan. 24, 2014 (JP) ..... 2014-011362

(51) **Int. Cl.**

**B23F 1/00** (2006.01)

**B22F 3/20** (2006.01)

**C22C 14/00** (2006.01)

**B22F 9/16** (2006.01)

**B22F 1/00** (2006.01)

**C22C 1/04** (2006.01)

**C23C 8/24** (2006.01)

(52) **U.S. Cl.**

CPC ..... **B22F 9/16** (2013.01); **B22F 1/0003**

(2013.01); **B22F 1/0088** (2013.01); **B22F 3/20**

(2013.01); **C22C 1/0458** (2013.01); **C22C**

**14/00** (2013.01); **C23C 8/24** (2013.01); **B22F**

**2201/02** (2013.01); **B22F 2301/205** (2013.01);

**B22F 2998/10** (2013.01)

(58) **Field of Classification Search**

CPC ..... C23C 8/24; C22C 1/0458; C22C 14/00;  
B22F 2201/02; B22F 1/0003; B22F  
1/0088; B22F 3/20; B22F 2301/205

See application file for complete search history.

(56) **References Cited**

U.S. PATENT DOCUMENTS

5,152,960 A \* 10/1992 Yuki ..... C22C 14/00  
148/407  
2012/0149183 A1 \* 6/2012 Kim ..... H01L 27/0688  
438/570  
2014/0212319 A1 \* 7/2014 Shiraishi ..... C22C 14/00  
419/13

FOREIGN PATENT DOCUMENTS

|    |                |           |
|----|----------------|-----------|
| EP | 0 457 340 A1   | 11/1991   |
| JP | 61-110734      | * 5/1986  |
| JP | 63-60296       | * 3/1988  |
| JP | 4-218634       | * 8/1992  |
| JP | 2009-280842 A  | 12/2009   |
| JP | 4408184 B2     | 2/2010    |
| JP | 2012-41609 A   | 3/2012    |
| JP | 2012-251234 A  | 12/2012   |
| JP | 2012-255192 A  | 12/2012   |
| WO | WO 2012/169305 | * 12/2012 |

OTHER PUBLICATIONS

International Search Report from corresponding International Application No. PCT/JP2014/084530.

Ando, Tomohiro, et al., "Effect of Nitrogen on Tensile Deformation Behavior and Development of Deformation Structure in Titanium," Journal of the Japan Institute of Metals and Materials, vol. 72, No. 12 (2008), pp. 949-954.

Liu, et al., "Surface hardening of Ti alloy by gas-phase nitridation: kinetic control of the nitrogen surface activity," Metallurgical and Materials Transactions, vol. 36A, Sep. 2005, pp. 1-6.

\* cited by examiner

Primary Examiner — C Melissa Koslow

(74) Attorney, Agent, or Firm — Hauptman Ham, LLP

(57) **ABSTRACT**

A method for producing titanium powder containing a solid-soluted nitrogen comprises the step of heating titanium powder comprised of titanium particles in a nitrogen-containing atmosphere to dissolve nitrogen atoms and form a solid solution of nitrogen atom in a matrix of the titanium particle.

**2 Claims, 4 Drawing Sheets**

FIG. 1

HEAT TREATMENT FOR DIRECT FORMATION  
OF SOLID SOLUTION OF NITROGEN

FIG. 2



FIG. 3



FIG. 4



FIG. 5



FIG. 6



FIG. 7



FIG. 8



## 1

**TITANIUM POWDER CONTAINING  
SOLID-SOLUTED NITROGEN, TITANIUM  
MATERIAL, AND METHOD FOR  
PRODUCING TITANIUM POWDER  
CONTAINING SOLID-SOLUTED NITROGEN**

## TECHNICAL FIELD

The present invention relates to titanium powder and titanium materials, and more particularly to titanium powder strengthened by a solid solution of nitrogen in titanium, titanium materials, and methods for producing such a strengthened titanium powder and a titanium material.

## BACKGROUND ART

Titanium is a lightweight material whose specific gravity is as low as about half that of steel and which is characterized by its high corrosion resistance and high strength. Titanium is therefore used for parts of aircrafts, railway vehicles, two-wheeled vehicles, automobiles, etc. for which reduction in weight is greatly desired, home appliances, members for construction, etc. Titanium is also used as a material for medical use because of its high corrosion resistance.

However, applications of titanium are limited due to its high material cost, as compared to iron and steel materials and aluminum alloys. In particular, titanium alloys have tensile strength as high as more than 1,000 MPa, but do not have enough ductility (elongation to failure). Moreover, titanium alloys have poor plastic workability at normal temperature or in a low temperature range. Pure titanium has elongation to failure as high as more than 25% at normal temperature and has excellent plastic workability in a low temperature range. However, pure titanium has tensile strength as low as about 400 to 600 MPa.

Various studies have been carried out in response to a very strong need for titanium having both high strength and high ductility and for reduction in material cost of titanium. In particular, many techniques of strengthening titanium by using relatively inexpensive elements such as oxygen and nitrogen rather than expensive elements such as vanadium, scandium, and niobium have been studied as related art in order to achieve cost reduction.

For example, Journal of the Japan Institute of Metals and Materials, Vol. 72, No. 12 (2008), pp. 949-954 (Non-Patent Literature 1), entitled "Effect of Nitrogen on Tensile Deformation Behavior and Development of Deformation Structure in Titanium," describes the use of nitrogen as an alloy element for titanium alloys. Specifically, Non-Patent Literature 1 describes that titanium sponge and TiN powder are weighed to predetermined compositions and are arc-melted to produce Ti—N alloys with various nitrogen concentrations. In this case, both high strength and high ductility can be achieved if a homogenous solid solution of nitrogen atoms in a Ti matrix is formed.

Another method is a technique of adding TiN particles to molten Ti to form a solid solution of nitrogen atoms in a Ti matrix when the mixture of TiN particles and molten Ti solidifies. In this case as well, both high strength and high ductility can be achieved if a homogenous solid solution of nitrogen atoms in the Ti matrix is formed.

## 2

## CITATION LIST

## Non-Patent Literature

- 5 NPL 1: Journal of the Japan Institute of Metals and Materials, Vol. 72, No. 12 (2008), pp. 949-954

## SUMMARY OF INVENTION

## Technical Problem

In conventional melting methods (in particular, a method of adding TiN particles to molten Ti), nitrogen atoms are significantly diffused and therefore are concentrated in the upper part of the molten Ti. Accordingly, it is difficult to uniformly disperse nitrogen in a large ingot, which significantly reduces ductility.

It is an object of the present invention to provide a method for producing titanium powder containing a solid-soluted nitrogen, in which nitrogen atoms can be uniformly diffused in a matrix of Ti particles to form a solid solution.

It is another object of the present invention to provide titanium powder and a titanium material which have both high strength and high ductility by uniformly diffusing nitrogen atoms in a matrix of Ti powder particles to form a solid solution.

## Solution to Problem

A method for producing titanium powder containing a solid-soluted nitrogen according to the present invention comprises the step of heating the titanium powder comprised of titanium particles in a nitrogen-containing atmosphere to dissolve nitrogen atoms and form a solid solution of the nitrogen atom in a matrix of the titanium particles. A heating temperature for forming the solid solution of the nitrogen atom in the matrix of the titanium particles is preferably 400° C. or more and 800° C. or less.

In the titanium powder containing the solid-soluted nitrogen produced by the above method, the titanium particle preferably has a nitrogen content of 0.1 mass % or more and 0.65 mass % or less. For reference, the nitrogen contents of four types of pure titanium specified by Japanese Industrial Standards (JIS) are as follows:

- JIS H 4600 Type 1: 0.03 mass % or less  
JIS H 4600 Type 2: 0.03 mass % or less  
JIS H 4600 Type 3: 0.05 mass % or less  
JIS H 4600 Type 4: 0.05 mass % or less

A titanium material is a material produced by forming the titanium powder containing the solid-soluted nitrogen into a predetermined shape. In one embodiment, the titanium material is an extruded material of pure Ti powder, the extruded material has a nitrogen content of 0.1 mass % to 0.65 mass %, and the extruded material has elongation to failure of 10% or more.

Examples of a method for compacting the titanium powder containing the solid-soluted nitrogen to produce the titanium material include powder compaction and sintering, hot extrusion, hot rolling, thermal spraying, metal injection molding, powder additive manufacturing, etc.

Functions and effects or technical significance of the above characteristic configuration will be described in the following sections.

## BRIEF DESCRIPTION OF DRAWINGS

FIG. 1 is a diagram schematically showing characteristics of the present invention.

FIG. 2 is a diagram showing data measured with a differential thermogravimetric analyzer.

FIG. 3 is a diagram showing diffraction peak shifts of Ti caused by heat treatment for formation of a solid solution of nitrogen.

FIG. 4 shows the measurement result of crystal orientation analysis (SEM-EBSD).

FIG. 5 is a diagram showing the relationship between stress and strain.

FIG. 6 is a diagram showing the relationship between heat treatment time and nitrogen and oxygen contents.

FIG. 7 is a diagram showing the relationship between nitrogen content and micro Vickers hardness Hv.

FIG. 8 is a diagram showing the relationship between proportion of the oxygen gas flow rate and nitrogen and oxygen contents.

#### DESCRIPTION OF EMBODIMENTS

FIG. 1 is a diagram schematically showing characteristics of the present invention. First, the outline of the present invention will be described with reference to FIG. 1, and more detailed data etc. will then be described.

##### [Preparation of Titanium Powder]

A titanium powder made of a multiplicity of titanium particles is prepared. As used herein, the "titanium particles" may be either pure titanium particles or titanium alloy particles.

##### [Heat Treatment for Solid Solution Formation]

The titanium powder comprised of titanium particles is heated in a nitrogen-containing atmosphere and retained therein to uniformly diffuse nitrogen atoms in a matrix of the titanium particles to form a solid solution, so that an intended solid solution of nitrogen in the titanium powder is eventually produced.

For example, heating conditions are as follows.

Heating atmosphere: 100 vol % of N<sub>2</sub> gas

Gas flow rate: 5 L/min

Heating temperature: 400 to 600° C.

Retention time: 1 to 2 hours

By the above heat treatment for solid solution formation, the nitrogen atoms are uniformly diffused in the matrix of the titanium powder particles to form a solid solution. Either a tubular heating furnace (non-rotary) or a rotary kiln furnace may be used because a sintering phenomenon between the titanium particles does not proceed in the above heating process.

For example, the titanium powder containing the solid-soluted nitrogen thus produced is compacted by powder compaction and sintering, hot extrusion, hot rolling, thermal spraying, metal injection molding, powder additive manufacturing, etc.

##### [Examination with Differential Thermogravimetric Analyzer (TG-DTA)]

Pure Ti raw material powder was placed into a furnace. With nitrogen gas being introduced into the furnace at a flow rate of 150 mL/min, the pure Ti raw material powder was heated from normal temperature to 800° C. (1,073 K). The weight started increasing at a temperature near 400° C. (673 K), and the weight subsequently significantly increased with an increase in temperature. The result is shown in FIG. 2. In FIG. 2, TG (Thermogravimetry) represents a change in weight and DTA (Differential Thermal Analysis) represents exothermic/endothermal behavior.

##### [Measurement of Nitrogen and Oxygen Contents]

With nitrogen gas being introduced into a tubular heating furnace at a flow rate of 5 L/min, pure Ti powder was heated

at 400° C. (673 K), 500° C. (773 K), and 600° C. (873 K) for one hour. Thereafter, the nitrogen content and the oxygen content in the resultant Ti powder were measured. The result is shown in Table 1.

TABLE 1

| Specimens                   | Nitrogen Content<br>(mass %) | Oxygen Content<br>(mass %) |
|-----------------------------|------------------------------|----------------------------|
| Pure Ti Raw Material Powder | 0.018                        | 0.270                      |
| 673K for 1 hr               | 0.041                        | 0.276                      |
| 773K for 1 hr               | 0.129                        | 0.275                      |
| 873K for 1 hr               | 0.292                        | 0.290                      |

Table 1 shows that the nitrogen content increased with an increase in heating temperature. However, the oxygen content changed very little. This shows that oxidation of the Ti powder in the heating process was restrained.

The result of Table 1 closely matches the result obtained by the differential thermogravimetric analyzer (TG-DTA). It is therefore desirable that the heating temperature be 400° C. (673 K) or more in order to form a solid solution of nitrogen atoms in a Ti matrix. However, the heating temperatures higher than 800° C. cause partial sintering between Ti particles. It is therefore desirable that the heating temperature be 800° C. or less.

##### [Examination with Diffraction Peaks]

FIG. 3 shows diffraction peak shifts of Ti caused by heat treatment for formation of a solid solution of nitrogen. Specifically, with nitrogen gas being introduced into a tubular heating furnace at a flow rate of 5 L/min, pure Ti powder was heated at 600° C. (873 K) for one hour and two hours. Thereafter, X-ray diffraction (XRD) analysis of the resultant Ti powder was conducted.

As can be seen from FIG. 3, diffraction peaks of Ti are shifted to lower angles if pure titanium raw material powder is subjected to the heat treatment for formation of a solid solution of nitrogen. These peak shifts show that a solid solution of nitrogen atoms in a Ti matrix was formed.

The oxygen and nitrogen contents in the above specimens were measured. The result is shown in Table 2.

TABLE 2

|                        | Nitrogen Content<br>(mass %) | Oxygen Content<br>(mass %) |
|------------------------|------------------------------|----------------------------|
| Raw Material Powder    | 0.018                        | 0.260                      |
| Powder Heated for 1 hr | 0.290                        | 0.263                      |
| Powder Heated for 2 hr | 0.479                        | 0.262                      |

The result of Table 2 shows that the oxygen content changed very little, and the nitrogen content increased with an increase in heating time.

##### [Examination with Crystal Orientation Analysis (SEM-EBSD)]

Each of the Ti powders was formed and compacted by spark plasma sintering. The resultant sintered body was hot-extruded to produce an extruded material with a diameter φ of 7 mm.

In the spark plasma sintering, each Ti powder was heated in a vacuum atmosphere at 800° C. for 30 min, and a pressure of 30 MPa was applied to each Ti powder in the heating process.

In the hot extrusion, the sintered body was heated in an argon gas atmosphere at 100° C. for 5 min. The heated



TABLE 6-continued

| Oxygen Gas Flow Rate (L/min)           | 0     | 0.06  | 0.15  | 0.24  | 0.3   | 0.45  | 0.6   | 0.75  |
|----------------------------------------|-------|-------|-------|-------|-------|-------|-------|-------|
| Proportion of Oxygen Gas Flow Rate (%) | 0     | 2     | 5     | 8     | 10    | 15    | 20    | 25    |
| Nitrogen Content (mass %)              | 0.518 | 0.512 | 0.519 | 0.522 | 0.514 | 0.491 | 0.465 | 0.433 |
| Oxygen Content (mass %)                | 0.225 | 0.232 | 0.236 | 0.242 | 0.246 | 0.278 | 0.292 | 0.319 |

As can be seen from FIG. 8 and Table 6, when the proportion of oxygen gas is 10 vol % or less, the oxygen content does not significantly increase, which shows that only nitrogen atoms are diffused in a Ti matrix to form a solid solution. However, when the proportion of oxygen gas is higher than 15 vol %, the oxygen content also increases, which shows that both nitrogen atoms and oxygen atoms can be diffused in a Ti matrix to form a solid solution. According to this production method, Ti powder in which not only nitrogen atoms but also oxygen atoms are diffused to form a solid solution can be produced by adjusting the mixing ratio of oxygen gas and nitrogen gas in a heat treatment atmosphere.

#### INDUSTRIAL APPLICABILITY

The present invention can be advantageously used to produce titanium powder strengthened by a solid solution of nitrogen in titanium and maintaining appropriate ductility by uniformly diffusing nitrogen in a matrix to form a solid solution, and a titanium material.

The invention claimed is:

1. A method for producing titanium powder containing a solid-soluted nitrogen, the method comprising:
  - heating titanium powder comprising titanium particles in a nitrogen-containing atmosphere to dissolve nitrogen atoms and form a solid solution of nitrogen atoms in a matrix of the titanium particles, wherein
  - a heating temperature for forming the solid solution of the nitrogen atoms in the matrix of the titanium particles is 400° C. or more and 600° C. or less, and the heating causes the titanium particles to have a nitrogen content of 0.1 mass % or more and 0.65 mass % or less.
2. The method for producing the titanium powder containing the solid-soluted nitrogen according to claim 1, wherein the heating of the titanium powder in the nitrogen-containing atmosphere occurs for a period of time corresponding to the heating temperature to cause the titanium particles in the matrix of titanium particles to have the nitrogen content of 0.1 mass % or more and 0.65 mass % or less.

\* \* \* \* \*